

## 1

3,021,232

## PROCESS FOR RENDERING SYNTHETIC HYDROPHOBIC MATERIAL ANTISTATIC AND THE PRODUCT OBTAINED THEREFROM

John Edward Pretka, Wilmington, Del., assignor to E. I. du Pont de Nemours and Company, Wilmington, Del., a corporation of Delaware  
No Drawing. Filed Nov. 17, 1958, Ser. No. 774,138  
13 Claims. (Cl. 117—138.8)

This invention relates to new compositions of matter. More particularly it is concerned with a synthetic, hydrophobic shaped structure bearing a novel finish to minimize the accumulation of charges of static electricity during finishing operations and normal use.

One common disadvantage of synthetic, hydrophobic shaped structures such as foams, fibers, filaments, yarns, staple, fabric, pellicles and the like, is that they tend to develop static electrical charges. This feature is objectionable during the manufacture of textiles and in the finished garment. During manufacturing, static charge from the fibers or fabric interferes with convenient handling during spinning, reeling, weaving, and the like operations. Finished textiles containing such structures fail to drape like cotton or wool due to their static charge and have a tendency to cling uncomfortably to the wearer. Furthermore such textiles tend to collect dust and lint. In addition, the electric discharge itself is bothersome. Most known antistatic agents useful in the textile arts lack durability and some impart to textiles undesirable properties such as unpleasant hand and discoloration upon application or with continued fabric use. Furthermore, some known antistatic agents are operable only within a narrow pH range and thus lack compatibility with many other common yarn-treating agents which are not stable in that pH range, making it necessary to apply the agent in a treatment step distinct from that employed for other purposes.

It is an object of the present invention to provide a composition which will impart durable antistatic protection to a synthetic, hydrophobic shaped structure without causing objectionable changes in other properties.

It is another object to provide a water-soluble antistatic composition which is compatible with pH sensitive yarn-finishing ingredients.

A further object is to provide a treated synthetic, hydrophobic shaped structure which minimizes or eliminates build-up of electrostatic charge and otherwise possesses substantially the same properties as the same structure before treatment.

Another object is to provide a process for imparting durable antistatic properties to a synthetic, hydrophobic shaped structure.

These and other objects will become apparent in the course of the following specification and claims.

In accordance with the present invention a synthetic, hydrophobic shaped structure which minimizes accumulation of charges of static electricity is provided by epoxide curing at a pH below 7.0 in the presence of an epoxide curing catalyst a synthetic hydrophobic shaped structure bearing a polyamine of the formula:



wherein  $-\text{R}-$  is a divalent radical,  $-\text{X}-$  is a member of the class consisting of amino nitrogen and divalent radical terminating in amino nitrogen,  $m$  and  $n$  are small whole numbers from about 3 to about 40 and  $p$  is an integer no greater than about 10. Since the nature of

## 2

$-\text{R}-$  is not critical provided it is inert to reaction with amines, it may be any member of the class consisting of



5 and  $-\text{A}-$  wherein  $-\text{A}-$  is a member of the class consisting of divalent aliphatic, alicyclic, aromatic and heterocyclic radicals. Preferably  $-\text{A}-$  is hydrocarbon. A particularly desirable class of polyamines are those of the formula:



wherein  $-\text{X}-$  is a member of the class consisting of



and



wherein  $-\text{R}'$  is a member of the class consisting of hydrogen, lower alkyl (i.e., an alkyl radical containing less than about 8 carbon atoms in its longest chain) and amino lower alkyl and  $-\text{Y}-$  is divalent aliphatic which while it may contain aza linkages is otherwise hydrocarbon,  $q$  being a number from about 6 to about 40. The preparation of these polyamines is discussed in detail in Belgian Patents 554,506, granted January 25, 1957, and

25 560,446, granted September 14, 1957. In general, the polyethylene glycol dihalide (e.g. chloride, bromide or iodide) analogue is condensed (with release of hydrogen halide) with an amine, the nitrogen of which contains at least two active hydrogen. Typical of such amines are

30 methylamine, ethylamine, propylamine, butylamine, amylamine, hexylamine, dodecylamine, alylamine, monoethanolamine, 3-isopropyl-n-propylamine, 3-methoxy-n-propylamine, diethylenetriamine, bis(3-aminopropyl)amine, bis(2-aminopropyl)amine, hexamethylene dia-

35 mine, triethylene tetramine, tetraethylene pentamine and the like. Such materials are available on the open market, typical products corresponding in general to Example 10 of Belgian Patent 560,446 and Example 1 of Belgian Patent 554,506. Assignee of the Belgian patent,

40 the Onyx Oil and Chemical Company of 115 Morris Street, Jersey City, New Jersey, markets such products under the trademarks Aston 108 and Aston LT.

45 By "epoxide curing" is meant that the polyamine defined above is reacted, after application of the reactants to the said shaped structure, with a polyepoxide. Such materials can be prepared by condensing epichlorohydrin with a polyol. A typical example is the condensation product (with elimination of HCl) of glycerine and epichlorohydrin. Preparation of these products is described in de-

50 tail in British Patent 780,288, dated July 31, 1957. Such a material with a molecular weight of between about 280 to 360 is available on the open market under the trademark "Eponite 100" (viscosity 90—150 cp. at 25° C.; 10.2 lbs./gal.) by the Shell Chemical Corp. of 500 Fifth Avenue, New York, N.Y. Other similar commercial products from the same source include the "Epon" resins which are diepoxy condensation products of epichlorohydrin and dimethyl, di-para hydroxyphenyl methane and the poly(allyl glycidyl ethers). A typical siloxane is 1,3-bis-

55 [3-(2,3-epoxy propoxy)propyl]tetramethylsiloxane sold under the trade mark "Syl-Kem 90" by Dow Corning Corp., Midland, Michigan. Reaction of the polyamine (I) or (II) with the polyepoxide may be conveniently accomplished by heating the shaped structure to which an

acidic mixture of the amine and polyepoxide has been applied.

In the examples which follow, unless otherwise stated, the "washed fabrics" are washed in a Kenmore portable washer at 140° F. using 0.125% "Tide" detergent in the presence of a small amount of trisodium hexametaphosphate, then thoroughly rinsed and dried. The dry cleaning operation employed involves a 25-minute tumble at room temperature using a solution of the following:

30 parts by volume perchloroethylene  
2.1 parts by volume dry cleaning soap (sold by R. R. Street & Co., Inc., 569 W. Monroe Street, Chicago, Illinois, under the trademark "Streets 886")  
0.2 part by volume water

After tumbling, the fabric is centrifuged for 6 minutes, tumbled for an additional 5 minutes with an equal amount of fresh, uncharged solvent, then centrifuged again for 5 minutes, dried for 2 minutes at from 60-70° C. and steam pressed. The bleaching procedure, representative of prevailing commercial practice, consists of immersing fabric in 100 times its weight of bleaching bath containing:

|                 | Percent |
|-----------------|---------|
| Sodium chlorite | .2      |
| Oxalic acid     | .2      |
| Nitric acid     | .11     |
| Sodium nitrate  | .5      |
| Water           | 99      |

heating to boiling, maintaining at boiling for 1 hour, and subsequently rinsing the fabric in warm water. The bleaching operation is then completed by a scour, i.e., boiling the fabric for 30 minutes in 100 times its weight of a detergent mixture consisting of:

|                       | Percent |
|-----------------------|---------|
| Green soap            | .1      |
| Sodium lauryl sulfate | .1      |
| Trisodium phosphate   | .1      |

followed by fabric rinsing, drying, and steam pressing.

Durability of antistatic treatments to bleaching, washing, and dry cleaning is determined by measurement of surface resistances of the fabrics. These measurements are made under controlled conditions of 25% relative humidity and a temperature of 70° F. Current flowing across the fabric is measured accurately with a Beckman, Model V Micro-microammeter, and the surface resistance is then calculated from this and the known applied voltage. For convenience, these values are reported as logarithms of surface resistance. In general, the lower the surface resistance, the lower is the tendency of the fabric to develop a static charge. Surface reflectance of undyed fabrics is used as a measure of whiteness. Measurements are made using a Photovolt Model 610 reflectometer. By using green, amber, and blue filters, grayness and yellowness can be estimated.

$$b_L = \frac{70(G-B)}{\sqrt{G}} \text{ (yellowness factor)}$$

where

B = reflectance with blue filter  
G = reflectance with green filter

The following examples are cited to illustrate the invention. They are not intended to limit it in any way. Unless otherwise noted, "parts" as expressed in the examples indicates parts by weight.

#### EXAMPLE 1

100 parts of the polyamine formed by condensation of diethylene triamine with the dichloride of polyethylene glycol having a molecular weight of 600 ("Aston LT" as identified above) as a 20% solids solution in water is stirred into 5000 parts of water. The pH of the resulting solution is adjusted to 3.2 by addition of 70 parts of a 10% solution of hydrochloric acid in

water. 62 parts of "Eponite 100" as identified above is then added and the mixture is dispersed using a Waring Blender. While mixing in the Waring Blender, 4 parts of zinc fluoroborate catalyst as a 40% aqueous solution is added. A slightly turbid solution is formed.

5 A swatch of tropical plain weave fabric woven from a polyethylene terephthalate yarn is dipped into the emulsion prepared as described above and squeezed between the rollers of a hand wringer. The fabric is then 10 cured for 5 minutes in an oven at 160° C. and thereafter scoured for 15 minutes at 140° F. The fabric is observed to have gained 3.2% by weight of antistatic finish based on the original weight of the fabric. The treated fabric has a log R of 10.3 compared with an 15 original log R of 14.2. After the standard bleaching the sample is observed to have a log R of 12.9.

A 21% by weight finish based on the weight of the fabric is attained when 1240 parts of "Eponite 100" is employed using the technique described above. In this 20 case 80 parts of the zinc fluoroborate catalyst is employed. The product has a log R of 11.0 before the standard bleaching and a log R of 11.5 after the bleaching.

#### EXAMPLE 2

Example 1 is modified by employing as the polyamine component the reaction product of the dichloride of polyethylene glycol having a molecular weight of 600 with methylamine ("Aston 108" as identified above). The percent by weight of finish picked up by the fabric samples as well as log Rs before and after standard bleaching when using 62 parts of the diepoxide (A) and when using 1240 parts of the diepoxide (B) are shown in Table I.

Table I

|   | Sample | Finish, Percent by wt. | Log R         |              |
|---|--------|------------------------|---------------|--------------|
|   |        |                        | Before Bleach | After Bleach |
| A |        | 2.8                    | 10.0          | 10.6         |
| B |        | 21.0                   | 10.7          | 11.7         |

Sample (B) is found to be waxy and stiff.

#### EXAMPLE 3

A Waring Blender is employed to mix 500 parts of "Aston 108" as a 20% solids solution in water, 100 parts of a 10% aqueous solution of hydrochloric acid, 62 parts of "Eponite 100" and 4 parts of zinc fluoroborate catalyst as a 40% aqueous solution. The pH of the resulting mixture is 3.5. The mixture is then stirred into 4340 parts of water. The finish is padded upon four fabric swatches identified in Table II.

Table II

|    | Sample | Identity                                                                                                                                                                   |
|----|--------|----------------------------------------------------------------------------------------------------------------------------------------------------------------------------|
| 60 | C      | Tropical plain weave from polyethyleneterephthalate yarn.                                                                                                                  |
|    | D      | Twill fabric woven from a yarn produced from a polymer of acrylonitrile ("Orlon," a trademarked product produced by E. I. du Pont de Nemours and Co. of Wilmington, Del.). |
| 65 | E      | Tricot fabric knitted with a polyhexamethylene-adipamide yarn.                                                                                                             |
|    | F      | Taffeta fabric woven from a polyhexamethylene-adipamide yarn.                                                                                                              |

The finish is applied using a laboratory padder set at 50 lbs. per square inch providing two dips and two nips. After padding all fabric samples are dried overnight at 70 room temperature and thereafter cured for 6 minutes at 150° C. The initial log R of the samples, the percent by weight of antistatic agent deposited based on the weight of the fabric and the log R observations before and after washing, bleaching and dry cleaning are shown 75 in Table III.

5  
Table III

| Sample | Log R<br>(Untreated) | Amount<br>Antistat.<br>(Percent<br>OWF) | Log R Treated           |      |      |             |                |
|--------|----------------------|-----------------------------------------|-------------------------|------|------|-------------|----------------|
|        |                      |                                         | After n Hrs.<br>Washing |      |      | 1<br>Bleach | 1 Dry<br>Clean |
|        |                      |                                         | 0                       | 5    | 23   |             |                |
| C      | 14.2                 | 0.9                                     | 11.2                    | 10.9 | 10.9 | 10.8        | 12.7           |
| D      | >16.3                | 2.5                                     | 10.3                    | 10.6 | 10.2 | 10.5        | 12.6           |
| E      | >16.3                | 1.1                                     | 11.9                    | 12.1 | 12.3 | 11.9        | 13.6           |
| F      |                      | 1.2                                     | 11.7                    | 12.7 | 12.6 | 11.3        | 13.2           |

For comparative purposes swatches of sample fabrics C, D and E above are padded with a solution containing 106 parts of water, 175 parts of an aqueous solution containing 35 parts "Aston 108" and 17 parts of a 90% aqueous solution of the diiodide of polyethylene glycol having a molecular weight of 600. The pH is adjusted with sodium hydroxide to 11.1. After drying at 212° F. fabrics are cured for about 3 minutes at 300° F. and thereafter scoured. The amount of finish pickup and the log R before and after and combination of one bleach and one scour are shown in Table IV. Comparative figures for similar samples treated in accordance with the present invention are included in the table. The samples treated with the finish cross-linked with the "diiodide" are labeled C<sub>1</sub>, D<sub>1</sub> and E<sub>1</sub>. In addition the table shows a comparative figure of yellowness factor relative to samples C and C<sub>1</sub>, D and D<sub>1</sub>. These compare to the yellowness factor of the untreated controls of 2.02 and 5.8 respectively.

Table IV

| Sample         | Amount<br>Antistat.<br>(Percent<br>OWF) | Log R   |                      |                      |
|----------------|-----------------------------------------|---------|----------------------|----------------------|
|                |                                         | Initial | 1 Bleach,<br>1 Scour | Yellowness<br>Factor |
| C              | 0.9                                     | 11.2    | 10.6                 | 4.07                 |
| C <sub>1</sub> | 2.4                                     | 11.4    | 13.5                 | 9.87                 |
| D              | 2.5                                     | 10.3    | 10.4                 | 6.94                 |
| D <sub>1</sub> | 2.4                                     | 9.7     | 14.3                 | 10.2                 |
| E              | 1.1                                     | 11.9    | 12.4                 | -----                |
| E <sub>1</sub> | 2.0                                     | 13.0    | 13.9                 | -----                |

## EXAMPLE 4

Solutions are made by adding 10 parts of the polyamine of Example 2 as a 20% solids solution in water to 1000 parts of water containing 2.5, 6.2 and 12.3 parts respectively, of "Epon" Resin 562, a condensation product of epichlorhydrin and glycerine containing 2 epoxy groups per molecule. To serve as control solutions, "Epon" Resin 562 is omitted from one solution of polyethylene glycol amine, and similarly, a 1% solution of "Epon" Resin 562 is prepared, omitting the polyamine. All solutions are acidified to pH 2.5 with HCl, including a pure water control containing no other ingredients. Samples of a tow of continuous filaments formed from a polymer of acrylonitrile (i.e. "Orlon" as identified above) are dipped into the test solutions at room temperature, wrung out to a solution pick-up of 100% and cured in a drying oven at 270° F. for ten minutes. The cured tow is converted into staple pads suitable for washing and testing for antistatic properties.

In this example in determining the durability of the antistatic properties, washing tests are carried out with 0.1% aqueous "Tide" using a 15-minute wash cycle at 60° C. followed by two 5 minute rinses at 60° C.

To determine the durability of the antistatic properties to dry cleaning, quarter-pound staple samples, wrapped in cheese cloth, are rolled for one-half hour in 13 pounds of Stoddard solvent containing 0.75% of dry cleaning soap (Streets 886 detergent). This is followed by two 15-minute rinses with pure Stoddard solvent, centrifuging after each rinse, and air drying.

6  
Table V

| Sample | Finishing Soln.<br>Compn. (per 1000<br>cc. H <sub>2</sub> O) | Log R                             |                           |                            |                             |                             |
|--------|--------------------------------------------------------------|-----------------------------------|---------------------------|----------------------------|-----------------------------|-----------------------------|
|        |                                                              | "Epon"<br>Resin<br>562<br>(parts) | Poly-<br>amine<br>(parts) | 1<br>wash                  | 5<br>washes                 | 10<br>washes                |
|        |                                                              |                                   |                           | 5<br>dry<br>clean-<br>ings | 10<br>dry<br>clean-<br>ings | 15<br>dry<br>clean-<br>ings |
| G      | 0                                                            | 10                                | 14.5                      | 14.7                       | -----                       | 14.3                        |
| H      | 2.5                                                          | 10                                | 10.9                      | 13.1                       | 13.9                        | -----                       |
| I      | 6.2                                                          | 10                                | 10.7                      | 13.4                       | 13.8                        | -----                       |
| J      | 12.3                                                         | 10                                | 10.4                      | 12.1                       | 12.9                        | 13.7                        |
| K      | 12.3                                                         | 0                                 | 14.6                      | -----                      | 14.3                        | 14.4                        |
| L      | 0                                                            | 0                                 | 14.7                      | -----                      | 14.5                        | 14.1                        |

15 A cationic blue tint when added to the compositions employed in treating samples H, I and J results in reduction of the color of the samples to less than that of the control. In a similar manner optical whiteners and silicone water proofing agents and other commonly used textile treating agents may be simultaneously applied with the antistatic agents of the present invention to perform their conventional roles.

20 Examples 1 and 2 are modified by employing as the curing agent 62 parts of "Syl-Kem 90" as identified above. The log R of the samples M and N respectively before scouring, after scouring and after 5 hours wash are reported in Table VI.

Table VI

| Sample | Pickup,<br>Percent<br>OWF | Log R           |                |                |
|--------|---------------------------|-----------------|----------------|----------------|
|        |                           | Before<br>Scour | After<br>Scour | 5 hrs.<br>Wash |
| M      | 2.9                       | 10.9            | 10.5           | 12.5           |
| N      | 3.1                       | 10.5            | 10.2           | 12.8           |

## EXAMPLE 6

45 A polyepoxide resin is prepared by mixing 15 parts of sodium styrene sulfonate, 80 parts of diionized water, 0.15 part of glyceryl monooleate, .08 part of alkyl phenoxyl polyoxyethanol and 1.67 parts of glycidyl methacrylate in a Waring Blender to form an emulsion. The emulsion is added to a 200 ml. 3-necked flask which is then flushed with nitrogen. .06 part of  $\alpha,\alpha$ -azobisisobutyryl nitrile is then added and the reaction mass is heated for 3 hours at 70° C. A thick semi-transparent emulsion is formed.

50 0.5 part of the polyamine, "Aston 108," is mixed with 0.5 part of the polyepoxide resin prepared as identified above to give an aqueous emulsion having 1% solids and the mixture is applied to staple fiber formed from a polymer of acrylonitrile (i.e. "Orlon" as identified above). The product is observed to have a  $b_L$  of 4.4. The log R values after 1, 5 and 10 washings (as described in Example 4) are listed below:

|             |      |
|-------------|------|
| 1 washing   | 10.7 |
| 5 washings  | 12.1 |
| 10 washings | 13.4 |

## EXAMPLE 7

65 The technique of Example 4 is followed in preparing three antistatic finish reactants (M, N and O) containing the polyamine and polyepoxide resin in a 1:1 weight ratio. Aston 108 is employed as the polyamine in each application. The emulsions are applied to a fabric woven from a polymer of acrylonitrile (i.e. "Orlon" as identified above) having an initial  $b_L$  of 3.0. The identity of the polyepoxide curing agent employed in each example is identified in Table VII. The color and log R of each sample after curing is reported in Table VIII.

7  
Table VII

| Sample | Polyepoxide Curing Agent   |
|--------|----------------------------|
| M..... | Eponite 100.               |
| N..... | Epon 815. <sup>1</sup>     |
| O..... | Poly allyl glycidyl ether. |

<sup>1</sup> A diepoxide condensation product of epichlorohydrin and dimethyl di-*para* hydroxyphenyl methane.

Table VIII

| Sample | b <sub>L</sub> | 1 Bleach | 5 Washes          | 10 Washes |
|--------|----------------|----------|-------------------|-----------|
| M..... | 4.8            | 13.3     | 13.1              | 13.6      |
| N..... | 3.9            | 13.6     | 13.9              | 13.9      |
| O..... |                |          | <sup>1</sup> 13.3 | 13.6      |

<sup>1</sup> Log R after one wash is 12.6.

## EXAMPLE 8

A mixture of 50 parts of "Aston 108" (20% active ingredients), 10 parts "Eponite 100" and 940 parts water is made up and adjusted to pH 3.5. A tow formed from a polymer of acrylonitrile (i.e. "Orlon" as identified above) is treated to provide a 100% by weight wet pickup of this solution, then cut into staple and dried at 270° F. for ten minutes. 20 parts of this treated staple is then blended with 80 parts untreated staple and the blend is spun into yarn and woven into a twill fabric. Samples of the fabric are washed, tested, bleached, disperse dyed and basic dyed. All exhibit static protection after 10 washes as shown in Table IX.

Table IX

| Sample                     | b <sub>L</sub><br>After 10<br>washes | Log R           |                    |                             |
|----------------------------|--------------------------------------|-----------------|--------------------|-----------------------------|
|                            |                                      | After 1<br>wash | After 10<br>washes | After 5<br>dry<br>cleanings |
| greige fabric.....         | 4.9                                  | 12.5            | 12.7               | 13.7                        |
| bleached fabric.....       | 0.7                                  | 12.6            | 13.0               | .....                       |
| disperse dyed fabrics..... |                                      | 12.8            | 13.3               | .....                       |
| basic dyed fabrics.....    |                                      | 12.6            | 12.9               | .....                       |
| cotton wool.....           |                                      |                 | 13.3               | 13.7                        |
| wool.....                  |                                      |                 |                    | 45                          |

By the expression ". . . synthetic, hydrophobic shaped structure . . ." is meant a structure such as a foam, fiber, filament, yarn, staple, fabric, pellicle and the like, produced from a synthetic polymeric material, having a moisture regain of no greater than 5%, such as a polyamide, a polymer produced from acrylonitrile, a polyester, or the like. Suitable polyamides are those produced from a linear polymer containing recurring units of the formula:



wherein Z is a member of the class consisting of a divalent hydrocarbon radical and a divalent radical of the formula



wherein G and G' are divalent hydrocarbon radicals. Typical polyamides and processes for their production are described in United States Patents Nos. 2,071,250; 2,071,253 and 2,130,948.

The term "polymer of acrylonitrile" is intended to include any polymer of acrylonitrile including polyacrylonitrile (i.e., the homopolymer) wherein the acrylonitrile component constitutes about 85% or more of the polymer molecule calculated as  $\text{CH}_2=\text{CH}-\text{CN}$ . Many of the ethylenically unsaturated compounds which are suitable

as the minor constituent in forming useful copolymers with acrylonitrile are listed in United States Patents Nos. 2,837,501; 2,486,241 and 2,436,926.

The polyesters from which such structures may be devised include polyethylene terephthalate, polyethylene terephthalate copolymers prepared using polyethylene glycols such as polyethylene glycols having molecular weights of 150 to about 6,000, or polyethers such as the dicarboxymethyl acid of polytetramethylene oxide or the esters polytetramethylene oxide, polydioxalane, or polyesters prepared using other acids such as bibenzoic, isophthalic or ethylene-bis-p-oxybenzoic acids. Such materials are described in United States Patent No. 2,465,319.

Application of the antistatic finish of the present invention may be made to any form of the shaped structure including foams, fabric, yarn, tow, staple, films, plastic sheeting and the like.

As described previously, the shaped structure is treated with an emulsion of a mixture of a polyepoxide and a compound of Formula I. Generally the emulsion is prepared by dispersing the polyamine and the polyepoxide in water at room temperature with vigorous stirring. The concentration of reactants in the emulsion may vary widely. A concentration as high as 20% may be used. However, more dilute emulsions containing from about 1 to about 5% of reactants are generally preferred. Any such finishing suspension having a concentration suitable to provide from about a 0.3% to about a 5% solids pickup based on the dry material is satisfactory. The reaction product can be applied to the structure by conventional methods such as dipping, padding, brushing, spraying, and the like. After removal of excess liquid, by wringing in the case of a textile, it is usually convenient to dry and cure the structure in one operation.

In forming the mixture of reactants the proportion of components may vary over a wide range. Preferably the ratio of polyamine:polyepoxide is maintained within the limits of 10:3 to 10:7. Higher ratios of polyepoxide such as 1:1 may be used however, as illustrated in the examples. Larger amounts of the polyepoxide may be employed but generally result in a harsher hand.

While, as illustrated above, the reactants may be applied to the shaped structure without the presence of catalysts, it is preferred to include a minor amount of an epoxide curing catalyst. Such materials not only hasten the curing operation or permit curing at lower temperature, but also increase adherence of the antistatic agent to the structure. Such materials are well known in the art, as described, for instance in United States Patent No. 2,752,269. Although the reacted mixture may be either acidic or alkaline, alkaline conditions usually cause yellowing.

Optimum conditions of curing will depend upon the identity of the reactants, the identity of the textile and whether or not a catalyst is included. Room temperature is adequate for forming the cured antistatic finish when a catalyst is used. Generally, however, a temperature of at least about 240° F. is preferred to accomplish efficient drying of the textile. Usually temperature adjustment is made to permit curing and drying in a 3-minute interval. A temperature of about 212° F. to 250° F. is recommended for most textile materials. For operation in the absence of a catalyst a curing cycle of about 10 minutes at 270° F. is adequate.

While applicant does not wish to be bound by any particular theory of mechanism, it is believed that the curing operation is accomplished by reaction of the epoxide with free hydrogen on the nitrogen of the polyamine. Thus it has been observed that fabrics treated with polyamines containing high proportions of active hydrogen (Aston LT) are stiffened to a greater extent upon curing than those where the polyamine has less free hydrogen (Aston 108).

Many modifications of the above will be obvious to those skilled in the art without a departure from the inventive concept.

What is claimed is:

1. A process of minimizing the accumulation of charge of static electricity upon a synthetic, hydrophobic shaped structure which comprises applying to the said structure at a pH below 7.0 and in the presence of an epoxide curing catalyst, a mixture of a polyepoxide and a polyamine of the formula:



wherein  $-\text{R}-$  is an organic divalent radical,  $-\text{X}-$  is a member of the class consisting of amino nitrogen and divalent radical terminating in amino nitrogen,  $m$  and  $n$  are small whole numbers from about 3 to about 40 and  $p$  is an integer no greater than about 10 and thereafter reacting the said polyepoxide and the said polyamine together.

2. The process of claim 1 wherein the shaped structure is a textile.

3. A process of minimizing the accumulation of charge of static electricity upon a synthetic, hydrophobic shaped structure which comprises applying to the said structure at a pH below 7.0 and in the presence of an epoxide curing catalyst, a mixture of a polyepoxide and polyamine of the formula:



wherein  $-\text{X}-$  is a member of the class consisting of



and



wherein  $-\text{R}'$  is a member of the class consisting of hydrogen, lower alkyl and amino lower alkyl,  $-\text{Y}-$  is a member of the class consisting of divalent aliphatic hydrocarbon and aza containing alkylene,  $q$  is a number from about 6 to about 40 and  $p$  is an integer no greater than about 10

and thereafter reacting the said polyepoxide and the said polyamine together.

4. The process of claim 3 wherein the shaped structure is a textile.

5. The process of claim 1 wherein the said polyepoxide curing catalyst is zinc fluoroborate.

6. The process of claim 3 wherein



is



15 7. The process of claim 3 wherein



is divalent ethylene triamine.

20 8. The process of claim 2 wherein the said textile is a fabric.

9. The process of claim 2 wherein the said textile is a filament.

10. The process of claim 2 wherein the yarn of the 25 said textile is produced from a polymer of acrylonitrile.

11. The process of claim 2 wherein the yarn of the said textile is a polyamide.

12. The process of claim 2 wherein the yarn of the said textile is a polyester.

30 13. The process of claim 1 wherein at least about 0.3% solids based on the dry material of the epoxide cured polyamine is applied to the said structure.

#### References Cited in the file of this patent

#### UNITED STATES PATENTS

35 2,794,754 Schroeder ----- June 4, 1957

#### FOREIGN PATENTS

40 554,506 Belgium ----- Jan. 27, 1957